# EUROPEAN PATENT APPLICATION

(11) **EP 4 786 620 A1**
(43) Date of publication of application: **05.08.2026**
(21) Application number: 24872558.2
(22) Date of filing: 27.09.2024
(51) Int. Cl.: C22C 38/00, C21D 8/12, C22C 38/60, H01F 1/16

(54) **GRAIN-ORIENTED ELECTRICAL STEEL SHEET AND MANUFACTURING METHOD THEREFOR**

(30) Priority: 27.09.2023 JP 2023166134
(71) Applicant: Nippon Steel Corporation, Tokyo 100-8071 (JP)
(72) Inventor: MATSUBARA, Ryo, Tokyo 100-8071 (JP); KAWAMURA, Yusuke, Tokyo 100-8071 (JP); HONMA, Rei, Tokyo 100-8071 (JP); SUZUMA, Toshiyuki, Tokyo 100-8071 (JP)
(74) Representative: Vossius & Partner Patentanwälte Rechtsanwälte mbB
(86) International application number: PCT/JP2024/034794
(87) International publication number: WO 2025/070777

(57) **Abstract**

The grain-oriented electrical steel sheet is a grain-oriented electrical steel sheet having a surface on which a plurality of magnetic domain control treatment lines extending in a direction intersecting a rolling direction are formed, in which a magnetic domain image of the surface is defined as a first magnetic domain image, a magnetic domain image at the same position as that of the first magnetic domain image after grain-oriented electrical steel sheet is annealed so as to be retained at 800°C for 240 minutes or more, cooled to 200°C at an average cooling rate of 25°C/h or less, and then cooled to 50°C or less at an average cooling rate of 100°C/h or less, is magnetized to a magnetic flux density of 1.9 T or more by applying an AC magnetic field, and is demagnetized by attenuating the AC magnetic field is defined as a second magnetic domain image, and
when a region in which a spacing of magnetic domain walls derived from the second magnetic domain image is larger than a spacing of magnetic domain walls derived from the first magnetic domain image by 100 µm or more is defined as a first region, and other regions are defined as a second region, a linear density of the magnetic domain control treatment line in the second region in a unit of mm/mm² is smaller than a linear density of the magnetic domain control treatment line in the first region in a unit of mm/mm².

## Description

### TECHNICAL FIELD

The present invention relates to a grain-oriented electrical steel sheet and a method for manufacturing the same.

The present application claims priority based on Japanese Patent Application No. 2023-166134 filed in Japan on September 27, 2023, the contents of which are incorporated herein by reference.

### BACKGROUND ART

The grain-oriented electrical steel sheet is a steel sheet containing 7 mass% or less of Si and having a secondary recrystallization texture in which secondary recrystallized grains are accumulated in a {110}<001> orientation (Goss orientation) in which an easy axis of magnetization <001> is oriented in a rolling direction. Grain-oriented electrical steel sheets are mainly used as iron cores of power transformers. Grain-oriented electrical steel sheets are required to reduce energy loss (iron loss).

A technique of narrowing a spacing of magnetic domain walls of a grain-oriented electrical steel sheet (magnetic domain refinement technique by magnetic domain control treatment) for reducing iron loss has been known. The spacing of magnetic domain walls can be narrowed by irradiating the surface of the grain-oriented electrical steel sheet with a laser or an electron beam in a direction intersecting the rolling direction to introduce a thermal strain. The spacing of magnetic domain walls can also be narrowed by forming a groove in the direction intersecting the rolling direction on the surface of the grain-oriented electrical steel sheet. Examples of a method of forming the groove include a method of irradiating a laser or an electron beam, a method by mechanical processing such as gear, and a method by chemical processing such as etching.

In recent years, in order to provide a grain-oriented electrical steel sheet having good iron loss characteristics, various improved techniques related to magnetic domain refinement have been proposed (see, for example, Patent Documents 1 to 3.).

In addition, in Patent Document 4, even in a case where local strain is applied for magnetic domain refinement, there are problems such as a decrease in magnetic permeability due to this strain, an increase in magnetic strain and an increase in noise, therefore a low-iron-loss grain-oriented electrical steel sheet in which problems such as a decrease in permeability and an increase in magnetostriction caused by linear grooves and local strain for magnetic domain refinement are reduced, and an advantageous method for manufacturing the same are proposed.

### Citation List

### Patent Documents

Patent Document 1: Japanese Unexamined Patent Application, First Publication No. 2012-57219
Patent Document 2: Japanese Unexamined Patent Application, First Publication No. 2012-12664
Patent Document 3: Japanese Unexamined Patent Application, First Publication No. 2012-57218
Patent Document 4: Japanese Unexamined Patent Application, First Publication No. H11-293340

### SUMMARY OF INVENTION

### Technical Problem

When the magnetic domain control treatment is applied to the grain-oriented electrical steel sheet, the magnetostrictive characteristic of the grain-oriented electrical steel sheet changes depending on the reflux magnetic domain. As a result, noise characteristics of the grain-oriented electrical steel sheet deteriorate. The noise characteristic is a degree of noise generated by an electrical product (for example, a transformer, a motor, and the like) manufactured using a grain-oriented electrical steel sheet as a material. Magnetostriction is a phenomenon in which an outer shape is slightly deformed when a ferromagnetic material is magnetized. When the grain-oriented electrical steel sheet is excited by alternating current, the magnitude of the magnetostriction changes with a change in the strength of magnetization, and thus vibration occurs. The magnitude of the magnetostriction is very small on the order of 10⁻⁶, but the magnetostriction generates vibration in the iron core, and the vibration propagates to an external structure such as a tank of a transformer to become noise. That is, the magnetic domain control treatment is effective for reducing iron loss of the grain-oriented electrical steel sheet, but deteriorates noise characteristics of the grain-oriented electrical steel sheet.

In recent years, there is an increasing demand for not only a reduction in iron loss but also a reduction in noise for grain-oriented electrical steel sheets. However, no magnetic domain refinement technique capable of sufficiently achieving both noise reduction and iron loss reduction has been proposed so far.

Further, in Patent Document 4, although noise is mentioned, both noise reduction and iron loss reduction cannot be sufficiently achieved. Patent Document 4 discloses that the β angle in the vicinity of the center in the rolling direction of the grain is 0° on average, and it is possible to achieve both noise reduction and iron loss reduction by applying the magnetic domain control treatment only to the region where the iron loss reduction effect by the magnetic domain control is large. However, there is also a result that the spacing of magnetic domain walls in each grain is substantially the same in the grain, and β angle near the center in the rolling direction of the grain is not necessarily 0°, both noise reduction and iron loss reduction cannot be sufficiently achieved even if the magnetic domain control treatment is performed by the method disclosed in Patent Document 4.

An object of the present disclosure is to provide a grain-oriented electrical steel sheet having a low iron loss (low iron loss) and a low noise (excellent noise characteristics) when the grain-oriented electrical steel sheet is made into an electrical product, and a method for manufacturing the grain-oriented electrical steel sheet. Solution to Problem

The present inventors have studied a grain-oriented electrical steel sheet having a low iron loss and excellent noise characteristics. As a result, it has been found that the magnetic domain control treatment is effective for reducing the iron loss of the grain-oriented electrical steel sheet, but deteriorates the noise characteristics of the grain-oriented electrical steel sheet, so that the deterioration of the noise characteristics can be suppressed by providing the non-magnetic domain control region.

The present invention has been made in view of the above findings.
[1] A grain-oriented electrical steel sheet according to one aspect of the present disclosure is a grain-oriented electrical steel sheet having a surface on which a plurality of magnetic domain control treatment lines extending in a direction intersecting a rolling direction are formed, wherein a magnetic domain image of the surface is defined as a first magnetic domain image, a magnetic domain image at the same position as that of the first magnetic domain image after the grain-oriented electrical steel sheet is annealed so as to be retained at 800°C for 240 minutes or more, cooled to 200°C at an average cooling rate of 25°C/h or less, and then cooled to 50°C or less at an average cooling rate of 100°C/h or less, is magnetized to a magnetic flux density of 1.9 T or more by applying an AC magnetic field, and is demagnetized by attenuating the AC magnetic field is defined as a second magnetic domain image, and when a region in which a spacing of magnetic domain walls derived from the second magnetic domain image is larger than a spacing of magnetic domain walls derived from the first magnetic domain image by 100 µm or more is defined as a first region, and other regions are defined as a second region, the linear density of the magnetic domain control treatment line in the second region in mm/mm² is smaller than the linear density of the magnetic domain control treatment line in the first region in mm/mm².
[2] In the grain-oriented electrical steel sheet according to [1], a difference between the linear density of the magnetic domain control treatment line in the second region and the linear density of the magnetic domain control treatment line in the first region may be 0.20 mm/mm² or more.
[3] In the grain-oriented electrical steel sheet according to [1] or [2], the plurality of magnetic domain control treatment lines may be thermal strains, or grooves and the thermal strains.
[4] In the grain-oriented electrical steel sheet according to any one of [1] to [3], the plurality of magnetic domain control treatment lines may be thermal strains into which a tensile stress of 40 MPa or more is introduced.
[5] A method for manufacturing a grain-oriented electrical steel sheet according to another aspect of the present disclosure includes: a first magnetic domain image acquisition step of acquiring a magnetic domain image before magnetic domain control treatment on a surface of a grain-oriented electrical steel sheet; a spacing of magnetic domain walls distribution acquisition step of acquiring a distribution of a spacing of magnetic domain walls in the grain-oriented electrical steel sheet based on the magnetic domain image before magnetic domain control treatment obtained in the first magnetic domain image acquisition step; a magnetic domain control treatment line forming step of forming a magnetic domain control treatment line on the surface of the grain-oriented electrical steel sheet; a second magnetic domain image acquisition step of acquiring a magnetic domain image after magnetic domain control treatment on the surface of the grain-oriented electrical steel sheet on which the magnetic domain control treatment line is formed; a magnetic domain image comparison step of comparing the magnetic domain image before the magnetic domain control treatment with the magnetic domain image after the magnetic domain control treatment; and an additional magnetic domain control treatment line forming step of further forming a magnetic domain control treatment line on the surface of the grain-oriented electrical steel sheet after the magnetic domain image comparison step as necessary, wherein in the magnetic domain control treatment line forming step, the magnetic domain control treatment line is formed in a region where the spacing of magnetic domain walls is more than 500 µm based on the distribution of the spacing of magnetic domain walls obtained in the spacing of magnetic domain walls distribution acquisition step; and in the magnetic domain image comparison step, when a region in which a spacing of magnetic domain walls derived from the magnetic domain image before the magnetic domain control treatment is larger than a spacing of magnetic domain walls derived from the magnetic domain image after the magnetic domain control treatment by 100 µm or more is defined as a first region, and other regions are defined as a second region, the linear density of the magnetic domain control treatment line in the second region in a unit of mm/mm² is compared with the linear density of the magnetic domain control treatment line in the first region in a unit of mm/mm², and in the additional magnetic domain control treatment line forming step, the magnetic domain control treatment line is formed in the first region in a case where the linear density of the second region is equal to or larger than the linear density of the first region; and the second magnetic domain image acquisition step, the magnetic domain image comparing step, and the additional magnetic domain control treatment line forming step are repeated until the linear density of the magnetic domain control treatment line in the second region becomes smaller than the linear density of the magnetic domain control treatment line in the first region.
[6] **In** the method for manufacturing a grain-oriented electrical steel sheet, in the magnetic domain control treatment line forming step, the magnetic domain control treatment line may be formed by irradiation with a laser or an electron beam.

### Advantageous Effects of Invention

According to the above aspect of the present disclosure, it is possible to provide a grain-oriented electrical steel sheet having a low iron loss (low iron loss) and having a low noise (excellent noise characteristics) when the grain-oriented electrical steel sheet is made into an electrical product, and a method for manufacturing the grain-oriented electrical steel sheet.

### BRIEF DESCRIPTION OF DRAWINGS

[FIG. 1A] A schematic view illustrating an example of a grain-oriented electrical steel sheet according to the present embodiment.
[FIG. 1B] A schematic view illustrating an example of a grain-oriented electrical steel sheet according to the present embodiment.
[FIG. 2] A graph showing a relationship between the spacing of magnetic domain walls before laser irradiation and the spacing of magnetic domain walls after laser irradiation.
[FIG. 3A] A diagram illustrating an example of distribution of a spacing of magnetic domain walls of a grain-oriented electrical steel sheet before a magnetic domain refinement treatment.
[FIG. 3B] A diagram illustrating an example of distribution of a spacing of magnetic domain walls of a grain-oriented electrical steel sheet after a magnetic domain refinement treatment.
[FIG. 3C] A view illustrating an example of a magnetic domain image acquired by the image acquisition device.
[FIG. 3D] A view schematically illustrating FIG. 3C.
[FIG. 4] A block diagram illustrating an example of a hardware constitution of the image acquisition device.
[FIG. 5] A block diagram illustrating an example of a hardware constitution of an analysis device.
[FIG. 6] A schematic diagram illustrating an example of a constitution of a laser irradiation device.
[FIG. 7] A flowchart illustrating an example of a method for manufacturing a grain-oriented electrical steel sheet according to the present embodiment.
[FIG. 8] A schematic view showing a method of cutting out a plurality of partial regions from a magnetic domain image of a grain-oriented electrical steel sheet.
[FIG. 9] An example of a plurality of partial Fourier images obtained by applying two-dimensional Fourier transform to each of a plurality of partial regions cut out from a magnetic domain image of a grain-oriented electrical steel sheet.

### DESCRIPTION OF EMBODIMENTS

A grain-oriented electrical steel sheet according to an embodiment of the present disclosure (grain-oriented electrical steel sheet according to the present embodiment) and a method for manufacturing the same will be described.

As illustrated in FIG. 1A, a grain-oriented electrical steel sheet 1 according to the present embodiment is a grain-oriented electrical steel sheet in which a plurality of magnetic domain control treatment lines 11 extending in a direction intersecting a rolling direction RD is formed on a surface thereof.

In the grain-oriented electrical steel sheet 1 according to the present embodiment, a magnetic domain image on a surface is defined as a first magnetic domain image, a magnetic domain image at the same position as the first magnetic domain image after annealing, magnetization, and demagnetization are performed under predetermined conditions is defined as a second magnetic domain image, and when a region in which a spacing of magnetic domain walls derived from the second magnetic domain image is larger than a spacing of magnetic domain walls derived from the first magnetic domain image by 100 µm or more is defined as a first region 21, and other regions are defined as a second region 22, the linear density in a unit of mm/mm² of the magnetic domain control treatment line in the second region 22 is smaller than the linear density in a unit of mm/mm² of the magnetic domain control treatment line in the first region 21.

As described later, the grain-oriented electrical steel sheet 1 according to the present embodiment may have a forsterite film and/or an insulating coating on the surface of a steel sheet to become a base steel sheet.

Each will be described below. However, in a case where the grain-oriented electrical steel sheet includes a base steel sheet and a forsterite film and/or an insulating coating, the following provisions regarding the chemical composition, the magnetic domain control treatment line, and the spacing of magnetic domain walls are provisions regarding the base steel sheet. However, the provision regarding the sheet thickness is a provision regarding the entire grain-oriented electrical steel sheet including the base steel sheet, and the forsterite film and/or the insulating coating.

### [Grain-Oriented Electrical Steel Sheet]

### (Chemical Composition)

The chemical composition of the grain-oriented electrical steel sheet 1 is not limited as long as it is equivalent to that of the known grain-oriented electrical steel sheet 1. For example, the grain-oriented electrical steel sheet 1 can contain, as a chemical composition, Si: 2.50 to 7.00%, Mn: 0 to 1.00%, C: 0 to 0.085%, acid-soluble Al: 0 to 0.065%, N: 0 to 0.012%, Cr: 0 to 0.300%, Cu: 0 to 0.400%, P: 0 to 0.500%, Sn: 0 to 0.300%, Sb: 0 to 0.300%, Ni: 0 to 1.000%, S: 0 to 0.015%, Se: 0 to 0.015%, Bi: 0 to 0.020%, Nb: 0 to 0.030%, V: 0 to 0.030%, Mo: 0 to 0.030%, Ta: 0 to 0.030%, W: 0 to 0.030%, B: 0 to 0.080%, and Ti: 0 to 0.015% in mass%. The balance of the chemical composition includes Fe and impurities.

The chemical compositions of the grain-oriented electrical steel sheet 1 may be measured by a general analysis method of steel. For example, the chemical component may be measured using inductively coupled plasma-atomic emission spectrometry (ICP-AES). Specifically, the chemical composition of the grain-oriented electrical steel sheet 1 can be measured by collecting a test piece from the center portion in the thickness direction of the sample, and measuring the test piece under a condition based on a calibration curve prepared in advance using ICPS-8100 manufactured by Shimadzu Corporation or the like (measuring device). The amounts of C and S, which are difficult to measure by ICP-AES, may be measured using a combustion-infrared light absorption method. The amount of N may be measured using an inert gas fusion-thermal conductivity method.

In a case where the forsterite film and/or the insulating coating are/is formed on the grain-oriented electrical steel sheet 1, the chemical composition of the grain-oriented electrical steel sheet 1 (that is, the chemical composition of the base steel sheet) may be analyzed after removing the forsterite film and/or the insulating coating from the grain-oriented electrical steel sheet 1.

The insulating coating can be removed, for example, by immersing the sample in a sodium hydroxide solution and then immersing the sample in dilute sulfuric acid and nitric acid. Conditions such as the temperature and concentration of sodium hydroxide, dilute sulfuric acid, and nitric acid solution, and the time for immersion are appropriately adjusted so that the base metal of the sample is not excessively dissolved. An example of the conditions of the removal operation of the insulating coating is as follows. First, the sample is immersed in a sodium hydroxide solution having a concentration of 20% at 80°C for 15 minutes. Thereafter, the sample is dried. Then, the sample is immersed in diluted sulfuric acid having a concentration of 10% at 80°C for 4 minutes. Thereafter, the sludge adhering to the surface of the sample is removed with a waste cloth or the like. Further, the sample is immersed in nitric acid having a concentration of 10% at room temperature while being stirred for about 10 seconds.

The forsterite film can be removed, for example, by immersing the sample in sulfuric acid followed by immersion in nitric acid. Conditions such as the temperature and concentration of sulfuric acid and nitric acid and the time for immersion are appropriately adjusted so that the base metal of the sample is not excessively dissolved. An example of conditions of the removal operation of the forsterite film is as follows. First, the sample is immersed in sulfuric acid having a concentration of 10% at 80°C for 3 minutes. Thereafter, the surface of the sample is washed with water using a waste cloth or the like to remove the sludge adhering to the surface. Thereafter, the sample is dried. Further, the sample is immersed in nitric acid having a concentration of 10% at room temperature while being stirred for about 5 seconds.

The sheet thickness of the grain-oriented electrical steel sheet 1 is not limited, but is preferably 0.15 mm to 0.30 mm, for example. When the sheet thickness is 0.30 mm or less, classical eddy-current loss can be suppressed, and iron loss can be further reduced. On the other hand, when the sheet thickness is 0.15 mm or more, rolling efficiency can be improved to improve productivity.

### (Magnetic domain control treatment line 11)

In the grain-oriented electrical steel sheet 1 according to the present embodiment, the plurality of magnetic domain control treatment lines 11 extending in the direction intersecting the rolling direction are formed on the surface.

The magnetic domain control treatment line 11 provided on the surface of the grain-oriented electrical steel sheet 1 has a function of refining a 180° magnetic domain. By refining the magnetic domain, the iron loss of the grain-oriented electrical steel sheet 1 can be reduced. The magnetic domain is a collection of magnetic dipoles existing inside a ferromagnetic material, and is a small region where magnetic moments are aligned in one direction. The 180° magnetic domain is a magnetic domain in which the magnetization direction is the <100> orientation of the crystal and which is sandwiched between two 180° magnetic walls substantially parallel to the rolling direction RD. A distance (domain wall interval) between adjacent domain walls of the 180° magnetic domain is referred to as a spacing of the 180° magnetic domain walls. Hereinafter, unless otherwise specified, the spacing of the 180° magnetic domain walls is simply referred to as "spacing of magnetic domain walls".

The extending direction of the magnetic domain control treatment line 11 is not particularly limited as long as it is a direction intersecting the rolling direction (as long as it is not parallel to the rolling direction). The magnetic domain control treatment line 11 and the rolling direction RD may be substantially perpendicular (substantially parallel to the transverse direction TD). That is, the angle formed by the magnetic domain control treatment line 11 and the transverse direction TD may be substantially 0°. On the other hand, as illustrated in FIG. 1A, the angle formed by the magnetic domain control treatment line 11 and the transverse direction TD may be more than 0°. For example, the angle formed by the magnetic domain control treatment line 11 and the transverse direction TD may be an arbitrary value within the range of 0° to 45°. The angle formed by the magnetic domain control treatment line 11 and the transverse direction TD may be 1° or more, 3° or more, or 5° or more. The angle formed by the magnetic domain control treatment line 11 and the transverse direction TD may be 40° or less, 35° or less, or 30° or less.

As illustrated in FIG. 1A, the angles formed by all the magnetic domain control treatment lines 11 and the transverse direction TD may be the same. That is, all the magnetic domain control treatment lines 11 may extend in parallel to each other. On the other hand, the angle formed by the magnetic domain control treatment line 11 and the transverse direction TD may vary. That is, some or all of a plurality of the magnetic domain control treatment lines 11 may extend non-parallel to each other. The average value of the angles formed by the magnetic domain control treatment line 11 and the transverse direction TD may be 1° or more, 3° or more, or 5° or more. The average value of the angles formed by the magnetic domain control treatment line 11 and the transverse direction TD may be 40° or less, 35° or less, or 30° or less. The average value of the angles may be calculated by measuring an angle formed with the transverse direction TD at a plurality of positions with respect to one magnetic domain control treatment line, or by measuring an angle formed with the transverse direction TD by a plurality of magnetic domain control treatment lines at one point or a plurality of positions.

In addition, as illustrated in Fig. 1B, the magnetic domain control treatment line 11 may include a curved portion (that is, may be constituted by only a straight line) or may be interrupted in the middle (that is, may be formed over the entire width direction of the steel sheet).

At least a part of the magnetic domain control treatment line 11 is the thermal strain. Since the thermal strain disappears by stress relief annealing or a heat treatment similar thereto, the spacing of magnetic domain walls changes before and after the heat treatment under predetermined conditions. A thermal strain and grooves or other magnetic domain control treatment lines may be used in combination.

In a case where the magnetic domain control treatment line 11 is a groove, the magnetic domain control treatment line 11 can be visually identified. In a case where the grain-oriented electrical steel sheet 1 has an insulating coating, the magnetic domain control treatment line 11 becomes visible by removing the insulating coating using a known peeling agent.

In a case where the magnetic domain control treatment line 11 is a thermal strain, the magnetic domain control treatment line 11 may not be visually identified. In this case, for example, the position of a thermal strain can be identified by photographing a magnetic domain image and observing the photographed magnetic domain image using the image acquisition device 30 having a constitution as show as an exemplary example in FIG. 4. At the time of photographing, as necessary, a magnetic domain image is photographed while a DC magnetic field is applied along the rolling surface normal direction ND of the grain-oriented electrical steel sheet 1.

### (Interval of magnetic domain control treatment line 11 along rolling direction RD)

In the plurality of magnetic domain control treatment lines 11, the interval along the rolling direction RD between the magnetic domain control treatment lines 11 adjacent along the rolling direction RD is not particularly limited. The effect of improving (reducing) the iron loss is enhanced as the interval is smaller. On the other hand, the larger the interval is, the more the noise characteristics are improved. The interval can be appropriately selected according to the characteristics required for the grain-oriented electrical steel sheet 1. For example, the interval along the rolling direction RD between the magnetic domain control treatment lines 11 adjacent to each other along the rolling direction RD may be 1.0 mm or more, 2.0 mm or more, 3.0 mm or more, or 5.0 mm or more. The interval along the rolling direction RD between the magnetic domain control treatment lines 11 adjacent along the rolling direction RD may be 10.0 mm or less, 9.0 mm or less, 8.0 mm or less, or 7.0 mm or less.

The interval of the adjacent magnetic domain control treatment lines 11 along the rolling direction RD may be constant or may vary (may fluctuate). In the case that variation is present, the average value of the interval along the rolling direction RD between the magnetic domain control treatment lines 11 adjacent to each other along the rolling direction RD may be 1.0 mm or more, 2.0 mm or more, 3.0 mm or more, or 5.0 mm or more. The average value of the intervals along the rolling direction RD between the magnetic domain control treatment lines 11 adjacent along the rolling direction RD may be 10.0 mm or less, 9.0 mm or less, 8.0 mm or less, or 7.0 mm or less. The interval may be obtained by drawing one or more straight lines L along the rolling direction RD and measuring the distance between two adjacent points LP at the intersection point LP of the straight line L and the magnetic domain control treatment line. In the case of calculating the average value of the intervals, a plurality of distances between two adjacent points LP may be measured and averaged.

The angle formed by the magnetic domain control treatment line 11 and the transverse direction TD can be measured using a known angle measuring means after the magnetic domain control treatment line 11 and the transverse direction TD are specified by the above-described and later-described procedures.

The interval of the magnetic domain control treatment line 11 along the rolling direction RD can be measured using a known length measuring means after the magnetic domain control treatment line 11 and the rolling direction RD are specified by the above-described and later-described procedures.

Here, the interval of the magnetic domain control treatment line 11 along the rolling direction RD is a distance from the center of the width of the magnetic domain control treatment line in the rolling direction RD to the center of the width of the adjacent magnetic domain control treatment line in the rolling direction RD.

As described above, at least a part of the magnetic domain control treatment line 11 is the thermal strain. That is, the magnetic domain control treatment line 11 is a thermal strain or other magnetic domain control treatment lines such as a thermal strain and a groove. The thermal strain can be formed using means such as laser irradiation, electron beam irradiation, and ion implantation. The groove can be formed using procedures such as laser irradiation, electron beam irradiation, machining, and etching.

In a case where the magnetic domain control treatment line is the thermal strain, it is preferable that tensile stress is introduced in the thermal strain. As the tensile stress is higher, the effect of reducing the iron loss is enhanced. On the other hand, the lower the tensile stress is, the more noise characteristics are improved. Tensile stress according to characteristics required for the grain-oriented electrical steel sheet 1 can be appropriately selected.

The magnitude of the tensile stress is not particularly limited, but for example, in at least a part of the magnetic domain control treatment line 11, the tensile stress in an arbitrary direction is preferably 40 MPa or more, 60 MPa or more, or 80 MPa or more. In a case where the tensile stress in at least one direction is 40 MPa or more, it is considered that the requirement that "the tensile stress in an arbitrary direction is 40 MPa or more" is satisfied. For example, in at least a part of the magnetic domain control treatment line 11, the tensile stress in an arbitrary direction is preferably 300 MPa or less, 200 MPa or less, 180 MPa or less, or 150 MPa or less. The tensile stress in an arbitrary direction in the magnetic domain control treatment line 11 may be uniform or may vary.

The magnitude of the tensile stress introduced in the thermal strain is measured by the EBSD Wilkinson method and Cross Court manufactured by BLG Vantage. The EBSD Wilkinson method is described in detail in A. J. Wilkinson, et al. "High-resolution elastic strain measurement from electron backscatter diffraction patterns: New levels of sensitivity" Ultramicroscopy Vol 106, No. 4-5, March 2006, P. 307-313.

When the magnitude of the tensile stress introduced in the thermal strain is measured by the EBSD Wilkinson method and the Cross Court manufactured by BLG Vantage, first, the magnetic domain control treatment line 11 is specified by the above-described procedure. Next, the grain-oriented electrical steel sheet 1 is cut through the magnetic domain control treatment line 11 and perpendicularly to the magnetic domain control treatment line 11. This cut cross section is used as a measurement surface. The cross section of the magnetic domain control treatment line 11 included in the measurement surface is analyzed by the EBSD Wilkinson method and Cross Court manufactured by BLG Vantage, and a tensile stress component in an arbitrary direction is extracted and the magnitude thereof is measured. For example, it is possible to extract a tensile stress component in a rolling surface normal direction ND, a direction parallel to the magnetic domain control treatment line 11, and a direction perpendicular to the rolling surface normal direction ND and the magnetic domain control treatment line 11.

The number of measurement points is, for example, 10. In a case where the tensile stress in an arbitrary direction is 40 MPa or more (that is, in a case where the tensile stress in at least one direction is 40 MPa or more) in at least one portion of the grain-oriented electrical steel sheet 1, the absolute maximum value of the tensile stress in an arbitrary direction in the magnetic domain control treatment line of the grain-oriented electrical steel sheet 1 is determined to be 40 MPa or more (The plurality of magnetic domain control treatment lines are the thermal strains into which a tensile stress of 40 MPa or more is introduced.). When a measurement point at which the tensile stress in any direction is 40 MPa or more is found, the measurement of the tensile stress may be stopped.

In the groove as the magnetic domain control treatment line, as the depth and width of the groove are larger, the effect of reducing the iron loss is enhanced. On the other hand, the noise characteristics are improved as the depth and width of the groove are smaller. The shape of the groove can be appropriately selected according to the characteristics required for the grain-oriented electrical steel sheet 1.

The depth of the groove is not particularly limited, but is preferably, for example, 5 µm to 50 µm. The depth of the groove may be 6 µm or more, 7 µm or more, or 10 µm or more. The depth of the groove may be 48 µm or less, 45 µm or less, or 40 µm or less.

The width of the groove (width at the opening part) is not particularly limited, but is preferably, for example, 10 µm to 300 µm. The width of the groove may be defined as 20 µm or more, 30 µm or more, or 50 µm or more. The width of the groove may be defined as 280 µm or less, 250 µm or less, or 200 µm or less. The depth and width of the groove may be uniform or may vary. In the case that variation is present, it is preferable that the average of the depths and widths of the plurality of grooves is within the above range.

The depth and width of the groove can be measured by specifying the surface shape of the sample using a known three-dimensional measuring machine. In a case where the grain-oriented electrical steel sheet 1 has an insulation coating, the insulating coating is removed by the above-described procedure, and then the three-dimensional measurement of the sample surface is performed.

### (Method for specifying rolling direction RD and transverse direction TD)

The rolling direction RD and the transverse direction TD of the grain-oriented electrical steel sheet 1 are specified by the following means.
(1) In a case where the sample is cut out from the coil-shaped grain-oriented electrical steel sheet 1, the width direction of the coil is regarded as the transverse direction TD. A direction perpendicular to the transverse direction TD and the rolling surface normal direction ND is regarded as the rolling direction RD.
(2) In a case where the sample is cut out from a part or the like of an electrical product, the rolling direction RD and the transverse direction TD are specified from rolling defects on the surface of the grain-oriented electrical steel sheet 1. The extending direction of the rolling defect is regarded as a rolling direction RD. A direction perpendicular to the rolling direction RD and the rolling surface normal direction ND is regarded as a transverse direction TD.
(3) In a case where it is difficult to specify the rolling direction RD and the transverse direction TD from a rolling defect on the surface of the grain-oriented electrical steel sheet 1, the rolling direction RD and the transverse direction TD are specified from the crystal orientation of the grain-oriented electrical steel sheet 1. Specifically, the crystal orientation of the grain-oriented electrical steel sheet 1 to be evaluated is measured at a plurality of points. Then, the direction in which the deviation angle from the easy axis of magnetization <001> at which the angle formed by the crystal orientation at the measurement point with the rolling surface normal direction ND (sheet thickness direction) is the closest to the right angle is minimized is regarded as the rolling direction RD, and the direction perpendicular to the rolling direction RD and the rolling surface normal direction ND is regarded as the transverse direction TD.

### (Spacing of magnetic domain walls)

In the grain-oriented electrical steel sheet according to the present embodiment, a magnetic domain image acquired from a surface is defined as a first magnetic domain image, a magnetic domain image at the same position as that of the first magnetic domain image after the temperature of the grain-oriented electrical steel sheet is retained at 800°C for 240 minutes or more, annealed to be cooled to 200°C at an average cooling rate of 25°C/h or less, and then cooled to 50°C or less at an average cooling rate of 100°C/h or less, magnetized to a magnetic flux density of 1.9 T or more by applying an AC magnetic field (magnetization is performed so that the magnetic flux density becomes 1.9 T), and demagnetized by attenuating the AC magnetic field is defined as a second magnetic domain image, and when a region in which a spacing of magnetic domain walls derived from the second magnetic domain image is larger than a spacing of magnetic domain walls derived from the first magnetic domain image by 100 µm or more is defined as a first region, and other regions are defined as a second region, the linear density (mm/mm²) of the magnetic domain control treatment line in the second region is smaller than the linear density (mm/mm²) of the magnetic domain control treatment line in the first region.

As described above, the magnetic domain control treatment line 11 provided on the surface of the grain-oriented electrical steel sheet 1 has a function of refining the 180° magnetic domain. Therefore, it is effective for reducing the iron loss of the grain-oriented electrical steel sheet.

On the other hand, the magnetic domain control treatment is effective for reducing the iron loss of the grain-oriented electrical steel sheet, but deteriorates the noise characteristics of the grain-oriented electrical steel sheet, so that the deterioration of the noise characteristics can be suppressed by providing the non-magnetic domain control region. That is, both noise reduction and iron loss reduction can be achieved in a well-balanced manner.

As a result of further studies, the present inventors have analyzed changes in the magnetic domains of the grain-oriented electrical steel sheets before and after the magnetic domain control, and as a result, it has become clear that there are portions where the spacing of magnetic domain walls is reduced and portions where the spacing of magnetic domain walls is hardly reduced by the magnetic domain control. That is, the present inventors have found that the magnetic domain refinement effect when the magnetic domain control treatment is performed differs depending on the spacing of magnetic domain walls before the magnetic domain control. More specifically, it has been found that the magnetic domain refinement effect by the magnetic domain control treatment is less likely to appear in a region having a narrow spacing of magnetic domain walls.

For example, as shown in Fig. 2, it has been found that there is an example in which the spacing of magnetic domain walls are substantially the same before and after the magnetic domain control treatment in a region where the spacing of magnetic domain walls before the magnetic domain control is about 500 µm or less, and the effect of the magnetic domain refinement by the magnetic domain control is hardly obtained in a region where the spacing of magnetic domain walls before the magnetic domain control is about 500 µm or less.

According to the above findings, it is found that it is extremely effective to preferentially perform a magnetic domain control treatment in a region having a wide spacing of magnetic domain walls in order to achieve both iron loss reduction and noise reduction. Magnetic domain control treatment in a region having a wide spacing of magnetic domain walls can reduce iron loss. A magnetic domain control treatment line formed in a region having a narrow spacing of magnetic domain walls is considered to cause deterioration of noise characteristics due to a flux closure domain. Therefore, deterioration of noise characteristics can be prevented by minimizing magnetic domain control treatment in a region having a narrow spacing of magnetic domain walls.

The grain-oriented electrical steel sheet according to the present embodiment is a grain-oriented electrical steel sheet in which a magnetic domain control treatment is selectively performed on a region having a wide spacing of magnetic domain walls and having a large magnetic domain refinement effect in order to obtain an effect of reducing iron loss while minimizing deterioration of noise characteristics. It is preferable to perform the magnetic domain control treatment only in a region having a wide spacing of magnetic domain walls, but it is allowable to perform the magnetic domain control treatment in a region having a narrow spacing of magnetic domain walls since the deterioration of noise characteristics is small if the ratio is small. In addition, it is preferable to perform the magnetic domain control treatment on all the regions with a wide spacing of magnetic domain walls, but a region where the magnetic domain control treatment is not performed may be included as long as the relationship of the linear density of the magnetic domain control treatment line after annealing is performed under the above-described predetermined conditions is satisfied.

However, in the grain-oriented electrical steel sheet after the magnetic domain control treatment, since the spacing of magnetic domain walls is narrow even in the region where the spacing of magnetic domain walls is wide, it is not easy to directly determine whether or not the magnetic domain control treatment has been performed only in the region where the magnetic domain refinement effect is large (it can be indirectly determined by noise characteristics and magnetic characteristics).

On the other hand, in the region where the spacing of magnetic domain walls was wide but the spacing of magnetic domain walls was narrowed by the formation of the magnetic domain control treatment line (by the magnetic domain control), when heat treatment such as stress relief annealing is performed, the effect of the magnetic domain control disappears, and the spacing of magnetic domain walls is widened (in the direction of returning to the original state). On the other hand, in a region where the spacing of magnetic domain walls is relatively narrow before the formation of the magnetic domain control treatment line, the spacing of magnetic domain walls is hardly widened even if the heat treatment such as stress relief annealing is performed.

That is, in the state of the grain-oriented electrical steel sheet not subjected to the stress relief annealing after the formation of the magnetic domain control treatment line, since there is no difference in the spacing of magnetic domain walls (The spacing of magnetic domain walls has become narrower overall.), the spacing of magnetic domain walls before the formation of the magnetic domain control treatment line cannot be determined. However, when the grain-oriented electrical steel sheet is subjected to stress relief annealing (or annealing corresponding thereto), it can be determined whether the region was a region having a wide spacing of magnetic domain walls (a region having a large magnetic domain refinement effect) or a region having a narrow spacing of magnetic domain walls (a region having a small magnetic domain refinement effect by magnetic domain control) before the magnetic domain control treatment line is formed.

In addition, by observing the change in the spacing of magnetic domain walls before and after the stress relief annealing and the formation position of the magnetic domain control treatment line, it can be determined whether the magnetic domain control treatment line is formed in a region having a large magnetic domain refinement effect or a region having a small magnetic domain refinement effect by the magnetic domain control. In other words, it is possible to determine whether or not the grain-oriented electrical steel sheet is a grain-oriented electrical steel sheet subjected to a magnetic domain control treatment for obtaining an effect of reducing iron loss while minimizing deterioration of noise characteristics.

The grain-oriented electrical steel sheet according to the present embodiment is a grain-oriented electrical steel sheet subjected to a magnetic domain control treatment for obtaining an effect of reducing iron loss while minimizing deterioration of noise characteristics. Specifically, as described above, a magnetic domain image of a surface is defined as a first magnetic domain image, a magnetic domain image at the same position as that of the first magnetic domain image after the temperature of the grain-oriented electrical steel sheet is retained at 800°C for 240 minutes or more, annealed to be cooled to 200°C at an average cooling rate of 25°C/h or less, and then cooled to 50°C or less at an average cooling rate of 100°C/h or less, which correspond to stress relief annealing, magnetized to a magnetic flux density of 1.9 T or more by applying an AC magnetic field, and demagnetized by attenuating the AC magnetic field is defined as a second magnetic domain image, and when a region in which a spacing of magnetic domain walls derived from the second magnetic domain image is larger than a spacing of magnetic domain walls derived from the first magnetic domain image by 100 µm or more is defined as a first region, and other regions are defined as a second region, the linear density of a magnetic domain control treatment line in the second region in of mm/mm² is smaller than the linear density of a magnetic domain control treatment line in the first region in of mm/mm².

The fact that the linear density of the magnetic domain control treatment line in the second region is smaller than the linear density of the magnetic domain control treatment line in the first region means that the magnetic domain control treatment line is formed mainly in a region having a wide spacing of magnetic domain walls (a region having a large magnetic domain refinement effect).

Preferably, a difference between the linear density of the magnetic domain control treatment line in the second region and the linear density of the magnetic domain control treatment line in the first region is 0.20 mm/mm² or more (That is, the linear density of the magnetic domain control treatment line in the second region - the linear density of the magnetic domain control treatment line in the first region ≤ -0.20 mm/mm².). In this case, the magnetic domain control treatment line is formed in a region having a wide spacing of magnetic domain walls (a region having a large magnetic domain refinement effect), so that the effect of reducing the iron loss can be obtained while further minimizing deterioration of noise characteristics.

The linear density of the magnetic domain control treatment line in the first region is preferably 0.05 mm/mm² or more, and more preferably 0.10 mm/mm² or more.

In addition, the linear density of the magnetic domain control treatment line in the second region is preferably 0.40 mm/mm² or less, and more preferably 0.20 mm/mm² or less. The linear density of the magnetic domain control treatment line in the second region may be 0.00 mm/mm².

In the region where the spacing of magnetic domain walls spread by the stress relief annealing is 100 µm or more, a certain degree of iron loss reduction effect is obtained by the magnetic domain control treatment. In addition, it is considered that the magnetic domain control treatment in the region where the spacing of magnetic domain walls spread by the stress relief annealing is less than 100 µm has a small iron loss reduction effect and deteriorates noise characteristics. Therefore, a region where the spacing of magnetic domain walls derived from the second magnetic domain image is 100 µm or more larger than the spacing of magnetic domain walls derived from the first magnetic domain image is defined as a first region.

The spacing of magnetic domain walls can be obtained by the following method.

For example, a sample having a side length of 100 mm (or 100 mm or more) can be cut out from the grain-oriented electrical steel sheet 1 and subjected to measurement. In a case where the grain-oriented electrical steel sheet 1 is a coil, a sample may be collected from an arbitrary position of the coil. In a case where the grain-oriented electrical steel sheet 1 is a component incorporated in an electrical product such as a transformer or a motor, a sample may be collected from any place of the component. In a case where the size of the component is small, the length of one side of the sample may be less than 100 mm. In this case, the total value of the sample areas is set to 10,000 mm² or more. At that time, it is desirable to collect a sample by a method such as wire cutting in order to minimize the influence of mechanical strain or the like on the sample. For this sample, a magnetic domain image (first magnetic domain image) is acquired by an image acquisition device including a light source unit, a magneto-optical sensor (MO sensor), an image sensor, and a signal processing unit. The magnetic domain image is output to an analysis device, which is a computer device such as a personal computer (PC) including a calculation unit, a memory, a display unit, an input unit, and a communication I/F, via a cable or by wireless communication. In the calculation unit, the magnetic domain structure is analyzed from the magnetic domain image using the line segment method.

An example of measurement by the line segment method will be described. FIG. 3C is a magnetic domain image acquired by CMOS-MagView manufactured by Matesy GmbH. FIG. 3D is a diagram schematically illustrating FIG. 3C for describing measurement.

In the line segment method, evaluation is performed by drawing a line segment Ls perpendicular to the magnetic domain. The interval between the line segments is drawn so as to be three per 1 cm in the rolling direction RD. The spacing of magnetic domain walls is derived based on the interval w of the intersection point Ip between the 180° magnetic domain wall and the line segment Ls. However, in a case where there are the flux closure domain 301 and the noise 302, these are not counted as domain walls. In a case where the average value of the spacings of magnetic domain walls is obtained, the average interval is obtained from the length of each line segment Ls and the number of intersection points Ip.

For the spacing of magnetic domain walls of the second magnetic domain image of the grain-oriented electrical steel sheet, a sample from which a first magnetic domain image is acquired is subjected to annealing in which the sample is retained at 800°C for 240 minutes or more and cooled to 200°C at an average cooling rate of 25°C/h or less and then 100°C/h or less to 50°C or less, and is magnetized to a magnetic flux density of 1.9 T or more by applying an AC magnetic field, and a magnetic domain image (second magnetic domain image) is acquired by an image acquisition device including a light source unit, a magneto-optical sensor (MO sensor), an image sensor, and a signal processing unit with respect to the sample demagnetized by attenuating the AC magnetic field. For this magnetic domain image, the spacing of magnetic domain walls can be measured in the same manner as described above.

The first region and the second region can be defined by comparing the spacing of magnetic domain walls derived from the obtained first magnetic domain image with the spacing of magnetic domain walls derived from the second magnetic domain image.

The linear density of the first region and the second region is obtained by the following method.

In the sample in which the spacing of magnetic domain walls is measured, the total length mm of the magnetic domain control treatment line included in each of the first region and the second region is measured, and the total length mm is divided by the area mm² of each region.

Measurement of any parameter described above is performed on a sample of a predetermined size collected from the grain-oriented electrical steel sheet 1. In a case where the grain-oriented electrical steel sheet 1 is a coil, a sample may be collected from an arbitrary position of the coil. In a case where the grain-oriented electrical steel sheet 1 is a component incorporated in an electrical product such as a transformer or a motor, a sample may be collected from any place of the component. In a case where the size of the component is small, the length of one side of the sample may be reduced, but the total value of the sample areas is set to be the same. In collecting the sample, it is desirable to collect the sample by a method such as wire cutting in order to minimize the influence of mechanical strain or the like on the sample.

### (Coating)

The grain-oriented electrical steel sheet 1 may have a forsterite film on its surface (That is, the grain-oriented electrical steel sheet may be composed of a base steel sheet and a forsterite film formed on the surface of the base steel sheet.). Further, the grain-oriented electrical steel sheet 1 may have an insulating coating on the surface of the base steel sheet or the surface of the forsterite film (That is, the grain-oriented electrical steel sheet may be composed of a base steel sheet, a forsterite film formed on the surface of the base steel sheet, and an insulating coating formed on the surface of the forsterite film, or may be composed of a base steel sheet and an insulating coating formed on the surface of the base steel sheet.).

The forsterite film and the insulating coating may be formed on one surface or both surfaces of the grain-oriented electrical steel sheet 1.

The forsterite film is, for example, an inorganic coating film containing magnesium silicate as a main component. The forsterite film is formed, for example, by a reaction between an annealing separator containing magnesia (MgO) applied to the surface of the base steel sheet and a component of the surface of the base steel sheet in final annealing. The forsterite film has, for example, a composition (more specifically, a composition containing Mg₂SiO₄ as a main component) derived from the components of the annealing separator and the base steel sheet. On the other hand, in a case where an annealing separator mainly containing Al₂O₃ is used in final annealing, a forsterite film may not be formed.

The insulating coating has a function of applying electrical insulation properties and tension to the grain-oriented electrical steel sheet 1. The tension is applied to the grain-oriented electrical steel sheet 1 to facilitate domain wall movement in the grain-oriented electrical steel sheet 1, and thus, the iron loss of the grain-oriented electrical steel sheet 1 can be reduced. In addition, according to the insulating coating, various characteristics such as corrosion resistance, heat resistance, and slippage can be provided to the grain-oriented electrical steel sheet 1. The insulating coating may be, for example, a known coating formed by applying a coating solution containing phosphate and colloidal silica as main components to the surface of the forsterite film and baking the coating solution.

### [Manufacturing Method]

The grain-oriented electrical steel sheet according to the embodiment exhibits its advantageous effects as long as it has the above characteristics, regardless of the manufacturing method therefor. However, according to the following method, it is preferable because it can be stably manufactured.

That is, the grain-oriented electrical steel sheet according to the present embodiment can be manufactured by a manufacturing method including the following steps (I) to (VI).
(I) A first magnetic domain image acquisition step of acquiring a magnetic domain image before magnetic domain control treatment on a surface of a grain-oriented electrical steel sheet;
(II) a spacing of magnetic domain walls distribution acquisition step of acquiring a distribution of a spacing of magnetic domain walls in the grain-oriented electrical steel sheet based on the magnetic domain image before magnetic domain control treatment obtained in the first magnetic domain image acquisition step;
(III) a magnetic domain control treatment line forming step of forming a magnetic domain control treatment line on the surface of the grain-oriented electrical steel sheet;
(IV) a second magnetic domain image acquisition step of acquiring a magnetic domain image after magnetic domain control treatment on the surface of the grain-oriented electrical steel sheet on which the magnetic domain control treatment line is formed;
(V) a magnetic domain image comparison step of comparing the magnetic domain image before the magnetic domain control treatment with the magnetic domain image after the magnetic domain control treatment; and
(VI) an additional magnetic domain control treatment line forming step of further forming a magnetic domain control treatment line on the surface of the grain-oriented electrical steel sheet after the magnetic domain image comparison step, as necessary.

Each step will be described.

First, the grain-oriented electrical steel sheet (original sheet) subjected to the first magnetic domain image acquisition step may be a known grain-oriented electrical steel sheet.

For example, the original sheet can contain, as a chemical composition, Si: 2.50 to 7.00%, Mn: 0 to 1.00%, C: 0 to 0.085%, acid-soluble Al: 0 to 0.065%, N: 0 to 0.012%, Cr: 0 to 0.300%, Cu: 0 to 0.400%, P: 0 to 0.500%, Sn: 0 to 0.300%, Sb: 0 to 0.300%, Ni: 0 to 1.000%, S: 0 to 0.015%, Se: 0 to 0.015%, Bi: 0 to 0.020%, Nb: 0 to 0.030%, V: 0 to 0.030%, Mo: 0 to 0.030%, Ta: 0 to 0.030%, W: 0 to 0.030%, B: 0 to 0.080%, and Ti: 0 to 0.015% in mass%. The balance of the chemical composition includes Fe and impurities.

A forsterite film may be formed on the surface of the grain-oriented electrical steel sheet serving as the original sheet.

### (First magnetic domain image acquisition step)

In the first magnetic domain image acquisition step, a magnetic domain image before magnetic domain control treatment on the surface of the grain-oriented electrical steel sheet is acquired.

As described later, in the method for manufacturing a grain-oriented electrical steel sheet according to the present embodiment, the magnetic domain control treatment lines are formed such that the linear density of the magnetic domain control treatment lines in the second region is smaller than the linear density of the magnetic domain control treatment lines in the first region. At that time, it is necessary to determine the first region and the second region. Therefore, in the first magnetic domain image acquisition step, a magnetic domain image before magnetic domain control treatment is acquired among magnetic domain images used for determining the first region and the second region.

The magnetic domain image can be acquired as described later.

### (Spacing of magnetic domain walls distribution acquisition step)

In the spacing of magnetic domain walls distribution acquisition step, a distribution of a spacing of magnetic domain walls (a distribution of a spacing of magnetic domain walls before a magnetic domain control treatment line is formed) in the grain-oriented electrical steel sheet is acquired based on the magnetic domain image before the magnetic domain control treatment obtained in the first magnetic domain image acquisition step.

Based on this distribution, in the magnetic domain control treatment line step, the position where the magnetic domain control treatment line is formed can be determined, and when the first region and the second region are determined in the magnetic domain image comparison step to be described later, the distribution of the spacing of magnetic domain walls derived from the reference magnetic domain image before magnetic domain control treatment can be obtained.

### (Magnetic domain control treatment line forming step)

In the magnetic domain control treatment line forming step, a plurality of magnetic domain control treatment lines extending in a direction intersecting the rolling direction are formed on the surface of the grain-oriented electrical steel sheet by mainly forming the magnetic domain control treatment lines in the region having the spacing of magnetic domain walls of more than 500 µm specified in the region specification step. As described above, it is considered that the effect of magnetic domain refinement is small in a region having a narrow spacing of magnetic domain walls, and the effect of magnetic domain refinement by magnetic domain control is hardly obtained in a region having a spacing of magnetic domain walls of about 500 µm or less. Therefore, it is preferable not to perform magnetic domain control in this region. It is preferable that the magnetic domain control treatment line is not formed in a region having a spacing of magnetic domain walls of 500 µm or less, but if the ratio is small, forming of the magnetic domain control treatment line is allowed. By forming the magnetic domain control treatment line, the spacing of magnetic domain walls in the vicinity thereof can be narrowed.

However, since this effect disappears by performing the stress relief annealing, in the region where the magnetic domain control treatment line due to the thermal strain is formed, the spacing of magnetic domain walls is widened by performing the stress relief annealing.

At least a part of the magnetic domain control treatment line is the thermal strain. Thermal strain and other magnetic domain control treatments such as grooves may be used in combination. In the case of the thermal strain, the magnetic domain control treatment line is formed by irradiation with a laser or an electron beam. Irradiation conditions may be in a known range.

Examples of forming the groove include a method of irradiating a laser or an electron beam, a method by mechanical processing such as gear, and a method by chemical processing such as etching.

The forming direction of the magnetic domain control treatment line (the scanning direction in the case of a laser or the like), the interval of the magnetic domain control treatment line in the rolling direction RD, the width of the magnetic domain control treatment line, and the depth in the case of a groove may be controlled by a known method so as to fall within the range of the grain-oriented electrical steel sheet according to the present embodiment described above.

### (Second magnetic domain image acquisition step)

In the second magnetic domain image acquisition step, a magnetic domain image after magnetic domain control treatment on the surface of the grain-oriented electrical steel sheet on which the magnetic domain control treatment line is formed is acquired. That is, a magnetic domain image after magnetic domain control treatment among magnetic domain images used for determining the first region and the second region is acquired.

The magnetic domain image can be acquired as described later.

At this stage, the distribution of the spacing of magnetic domain walls (the distribution of the spacing of magnetic domain walls after forming the magnetic domain control treatment line) in the grain-oriented electrical steel sheet may be acquired based on the obtained magnetic domain image after the magnetic domain control treatment.

### (Magnetic domain image comparison step)

In the magnetic domain image comparison step, when a region in which a spacing of magnetic domain walls derived from the second magnetic domain image is larger than a spacing of magnetic domain walls derived from the first magnetic domain image by 100 µm or more is defined as a first region, and other regions are defined as a second region, the linear density in mm/mm² of the magnetic domain control treatment line in the second region is compared with a linear density in mm/mm² of the magnetic domain control treatment line in the first region.

The linear density is calculated by measuring the total length mm of the magnetic domain control treatment line included in each of the first region and the second region and dividing the total length mm by the area mm² of each region.

As a result of the comparison of the linear densities, in a case where the linear density of the magnetic domain control treatment line in the second region is smaller than the linear density of the magnetic domain control treatment line in the first region, the additional magnetic domain control treatment line forming step, which is the next step, may not be performed.

On the other hand, as a result of the comparison of the linear densities, in a case where the linear density of the magnetic domain control treatment line in the second region is the same as the linear density of the magnetic domain control treatment line in the first region or larger than the linear density of the magnetic domain control treatment line in the first region, an additional magnetic domain control treatment line forming step which is a next step is performed.

### (Additional magnetic domain control treatment line forming step)

In the additional magnetic domain control treatment line forming step, in a case where it is determined in the magnetic domain image comparison step that the linear density of the magnetic domain control treatment line in the second region is the same as the linear density of the magnetic domain control treatment line in the first region or larger than the linear density of the magnetic domain control treatment line in the first region, the magnetic domain control treatment line is further formed in the first region to increase the linear density of the first region.

In the method for manufacturing a grain-oriented electrical steel sheet according to the present embodiment, the linear density of the magnetic domain control treatment line in the second region is made smaller than the linear density of the magnetic domain control treatment line in the first region.

However, at the stage of forming the magnetic domain control treatment line, the distribution of the spacing of magnetic domain walls of the first region and the second region after forming the magnetic domain control treatment line is unknown. Therefore, after the magnetic domain control treatment line is formed, the magnetic domain images before and after the magnetic domain control treatment line is formed are compared, and the linear density of the magnetic domain control treatment line between the first region and the second region is compared.

As a result, when the linear density of the magnetic domain control treatment line in the second region is smaller than the linear density of the magnetic domain control treatment line in the first region, the process ends. On the other hand, in a case where the linear density of the magnetic domain control treatment line is not smaller than the linear density of the magnetic domain control treatment line in the first region, an additional magnetic domain control treatment line forming step is further performed.

After the additional magnetic domain control treatment line forming step, the magnetic domain image after the magnetic domain control treatment on the surface of the grain-oriented electrical steel sheet on which the magnetic domain control treatment line is formed is acquired again (subjected to the second magnetic domain image acquisition step). Then, the magnetic domain image before the formation of the magnetic domain control treatment line and the magnetic domain image in the additional magnetic domain control treatment line forming step are compared, and the linear densities of the magnetic domain control treatment lines of the first region and the second region are compared.

As a result, when the linear density of the magnetic domain control treatment line in the second region is smaller than the linear density of the magnetic domain control treatment line in the first region, the process ends. On the other hand, in a case where the linear density is not yet smaller than the linear density of the magnetic domain control treatment line in the first region, the additional magnetic domain control treatment line forming step is performed again.

That is, the second magnetic domain image acquisition step, the magnetic domain image comparison step, and the additional magnetic domain control treatment line forming step are repeated until the linear density of the magnetic domain control treatment line in the second region becomes smaller than the linear density of the magnetic domain control treatment line in the first region.

That is, as shown in FIG. 7, a predetermined grain-oriented electrical steel sheet may be obtained by S1 -> S2 -> S3 -> S4 -> S5, but a predetermined grain-oriented electrical steel sheet may be obtained by S1 -> S2 -> S3 -> S4 -> S5 -> S6 -> S4 -> S5, and a predetermined grain-oriented electrical steel sheet may be obtained by S1 -> S2 -> S3 -> S4 -> S5 -> S6 -> S4 -> S5 -> S6 -> S4 -> S5. Furthermore, S4 -> S5 -> S6 may be repeated.

### (Specific method in magnetic domain image acquisition, spacing of magnetic domain walls distribution acquisition, and magnetic domain control treatment line formation)

The acquisition of the magnetic domain image and the acquisition of the distribution of the spacing of magnetic domain walls can be performed by the following method.

The magnetic domain image of the surface can be acquired by, for example, an image acquisition device. Next, the distribution of the spacing of the 180° magnetic domain walls (the spacing of magnetic domain walls) is derived from the magnetic domain image. The distribution of the spacing of magnetic domain walls in the original sheet can be derived by using, for example, an analysis device.

From the distribution of the spacing of magnetic domain walls, a region where the spacing of magnetic domain walls is a predetermined value or more (for example, a region where the spacing of magnetic domain walls is more than 500 µm, when a magnetic domain control treatment line is formed in a region where the spacing of magnetic domain walls is more than 500 µm in a subsequent step.) can be determined as a region where the magnetic domain control treatment is to be performed (hereinafter, simply referred to as a treatment region in some cases).

The treatment region may be determined by visually observing the magnetic domain image displayed on the display unit of the analysis device by the operator.

FIG. 4 illustrates an example of a hardware constitution of the image acquisition device 30 that acquires a magnetic domain image of an original sheet (grain-oriented electrical steel sheet 1 before magnetic domain control treatment). The image acquisition device 30 includes a light source unit 31, a magneto-optical sensor (MO sensor 33), an image sensor 35, and a signal processing unit 37.

The light source unit 31 includes a light source including a light emitting diode (LED), and irradiates the MO sensor 33 with light having a uniform polarization plane.

The MO sensor 33 is a device that measures a magnetic domain structure of a magnetic material. The MO sensor 33 has an observed section on which a magnetic sample to be measured is placed. The light irradiated from the light source unit 31 passes through the inside of the MO sensor 33 and is reflected by the reflection layer. The reflected light passes through the inside of the MO sensor 33 again and is output to the outside of the MO sensor 33. When the original sheet as a magnetic sample is placed on the observed section of the MO sensor 33, a leakage magnetic field corresponding to the direction of spontaneous magnetization of the original sheet is generated inside the MO sensor 33. This leakage magnetic field rotates the polarization plane of the reflected light.

The image sensor 35 is a Complementary Metal-Oxide-Semiconductor (CMOS) image sensor. The image sensor 35 forms an image of the reflected light from the MO sensor 33 on the light receiving surface to perform photoelectric conversion, and outputs an analog signal after the photoelectric conversion to the signal processing unit 37. The distribution of the leakage magnetic field can be obtained by detecting the reflected light in which the polarization plane is rotated by the image sensor 35, and the magnetic domain structure of the original sheet becomes clear.

The signal processing unit 37 includes an amplifier, an AD converter, a Digital Signal Processor (DSP), and the like. The analog signal output from the image sensor 35 is amplified by an amplifier. Then, the analog signal is converted into a digital signal by an AD converter. The digital signal is subjected to predetermined digital processing using a DSP to generate an image signal. The image signal generated by the signal processing unit 37 is output to the analysis device 40 (see FIG. 5) via a cable or by wireless communication.

FIG. 5 illustrates a hardware constitution of an analysis device 40 that analyzes the magnetic domain structure of the original sheet. The analysis device 40 is a computer device such as a personal computer (PC). The analysis device 40 includes a calculation unit 41, a memory 43, a display unit 45, an input unit 47, and a communication I/F 49.

The calculation unit 41 includes a Central Processing Unit (CPU). The calculation unit 41 analyzes the magnetic domain structure from the magnetic domain image of the original sheet according to the program stored in the memory 43. Then, the calculation unit 41 determines a treatment region to which the magnetic domain control treatment is applied. The processing executed by the calculation unit 41 is described in detail later.

The memory 43 includes a Read Only Memory (ROM) and a Random Access Memory (RAM). The ROM stores programs executed by the CPU of the calculation unit 41 and data required for executing these programs. The program and data stored in the ROM are loaded into the RAM and executed.

The memory 43 may include a magnetic memory such as a hard disk drive (HDD) or an optical memory such as an optical disk. Alternatively, the memory 43 may be detachable from the analysis device 40 and store programs and data in a computer-readable recording medium. Alternatively, the memory 43 may receive the program executed by the calculation unit 41 from the network via the communication I/F 49.

The display unit 45 includes a display such as a liquid crystal display (LCD), a plasma display, or an organic electroluminescence (EL) display. The display unit 45 displays an image on the basis of the image signal output from the image acquisition device 30. In addition, the display unit 45 displays the analysis result of the magnetic domain structure by the calculation unit 41.

The input unit 47 includes an input device such as a mouse or a keyboard. The communication I/F 49 is an interface for transmitting and receiving data to and from an external device via a network such as a Local Area Network (LAN), a Wide Area Network (WAN), or the Internet.

Instead of general-purpose hardware such as a CPU, dedicated hardware specialized for analyzing a magnetic domain structure, such as an application specific integrated circuit (ASIC) or a Field Programmable Gate Array (FPGA), may be adopted as the calculation unit 41.

FIGS. 4 and 5 illustrate a case where the image acquisition device 30 and the analysis device 40 are separate devices, but a system in which the image acquisition device 30 and the analysis device 40 are integrated may be adopted.

As means for introducing the thermal strain into the surface of the original sheet, known means such as laser irradiation, electron beam irradiation, and ion implantation can be adopted. As means for forming a groove on the surface of the original sheet, known means such as laser irradiation, electron beam irradiation, and machining can be adopted. Hereinafter, a constitution of the laser irradiation device 500 that introduces the thermal strain by laser irradiation will be described.

FIG. 6 illustrates a constitution of the laser irradiation device 500. The laser irradiation device 500 includes a polygon mirror 501, a light source device 503, a collimator 505, a condenser lens 507, a motor 509, a sensor 511, a control unit 513, and a sheet passing device 515.

The sheet passing device 515 passes the original sheet in the rolling direction RD.

The polygon mirror 501 has, for example, a regular polygonal prism shape. A plurality of the plane mirrors is provided on each of a plurality of side surfaces constituting the polygon mirror 501 having a regular polygonal prism shape. The laser beam LB enters the plane mirror of the polygon mirror 501 in one direction (horizontal direction) from the light source device 503 via the collimator 505 and is reflected by the plane mirror.

The polygon mirror 501 is rotatable about the rotary shaft O1 by driving from the motor 509. The incident angle of the laser beam LB with respect to the plane mirror sequentially changes according to the rotation angle of the polygon mirror 501. As a result, the reflection direction of the laser beam LB is sequentially changed, and the surface of the original sheet can be scanned. A Reference Sign P in FIG. 6 represents an interval between the adjacent magnetic domain control treatment lines 11, that is, an irradiation pitch of the laser beam LB.

The light source device 503 outputs the laser beam LB by a predetermined irradiation system (for example, a continuous irradiation system or a pulse irradiation system) under the control of the control unit 513.

The condenser lens 507 is provided on the optical path of the laser beam LB reflected from the polygon mirror 501. The condenser lens 507 constitutes a condenser optical system having a predetermined focal distance. The laser beam LB reflected from the polygon mirror 501 is condensed on the surface of the original sheet via the condenser lens 507, whereby the thermal strain is introduced into the surface of the original sheet.

The motor 509 is coupled to the polygon mirror 501. The motor 509 rotationally drives the polygon mirror 501 under the control of the control unit 513.

The sensor 511 is connected to a drive shaft of the motor 509. The sensor 511 detects a rotation angle of the polygon mirror 501 rotated by the motor 509. Furthermore, the sensor 511 outputs a signal (Hereinafter, the rotation angle signal is referred to as a rotation angle signal.) indicating the detected rotation angle to the control unit 513.

The control unit 513 includes a processor. The control unit 513 is connected to the light source device 503, the motor 509, the sensor 511, and the sheet passing device 515. The control unit 513 receives an input of a speed signal from the sheet passing device 515. Further, the control unit 513 outputs a signal instructing the motor 509 to rotationally drive the polygon mirror 501.

In addition, the control unit 513 controls on and off of the power of the laser beam LB output from the light source device 503 based on the stress introduction signal representing the treatment region and the rotation angle signal output from the sensor 511. In a case where the laser irradiation device 500 is electrically connected to the analysis device 40, the stress introduction signal is input from the analysis device 40 to the laser irradiation device 500. The stress introduction signal may be input to the laser irradiation device 500 by an operator.

Next, an example of a method of determining the treatment region will be described in detail. The processing for specifying the treatment region is executed by, for example, the calculation unit 41 of the analysis device 40.

The calculation unit 41 derives the distribution of the spacing of magnetic domain walls of the original sheet using, for example, a line segment method. Then, the calculation unit 41 determines a region where the spacing of magnetic domain walls is a predetermined value or more (for example, more than about 500 µm) as a portion to which the magnetic domain control treatment is preferentially applied.

In the line segment method, evaluation is performed by drawing a line segment perpendicular to the magnetic domain. The line segments are drawn at intervals of three lines per 1 cm in a direction parallel to the magnetic domain. A spacing of magnetic domain walls is derived based on an interval between the intersection points of 180° magnetic domain walls and line segments.

FIG. 3A illustrates an example of distribution of the spacing of magnetic domain walls of the grain-oriented electrical steel sheet 1 before the magnetic domain control treatment, which is obtained by further analyzing the magnetic domain image acquired by CMOS-MagView manufactured by Matesy GmbH by two-dimensional Fourier transform. FIG. 3B shows the distribution of the spacings of magnetic domain walls after the surface of the grain-oriented electrical steel sheet 1 of FIG. 3A is subjected to the magnetic domain control treatment, which is obtained in the same manner as in FIG. 3A. The magnetic domain control treatment here is performed by applying continuous wave laser irradiation along a direction substantially perpendicular to the rolling direction RD. In FIGS. 3A to 3B, the unit of the numerical value is µm.

As an example of analysis using the two-dimensional Fourier transform, a method for deriving a distribution of a spacings of magnetic domain walls is described using a short-interval two-dimensional Fourier transform (Hereinafter, it is referred to as "ST2DFT".) obtained by expanding a short-term Fourier transform, which is one of signal processing methods that have been used for time-frequency analysis of audio signals for a long time, to a two-dimensional region.

An image (magnetic domain image) represented by an image signal acquired by the image acquisition device 30 is expressed as x (k, l) as a data column of two-dimensional coordinates (k-l coordinates). In the present embodiment, the magnetic domain image to be analyzed is an image binarized with two types of colors or an image expressed in three or more gradations (multiple gradations) such as gray scale.

In order to derive the distribution of the spacings of magnetic domain walls of the original sheet 2, the calculation unit 41 executes the following processes (A-1), (A-2), and (A-3).
(A-1) Treatment of cutting out a plurality of partial regions from magnetic domain image;
(A-2) Treatment of performing ST2DFT;
(A-3) Treatment of deriving distribution of spacings of magnetic domain walls.

Hereinafter, the treatment of A-1 to A-3 will be described in detail.

### (A-1) Treatment of cutting out a plurality of partial regions from magnetic domain image

In order to cut out a plurality of partial regions from a magnetic domain image and analyze each frequency structure, a window function Wa (k, l) of a rectangular window in which a range in the k direction set to 0 ≤ k ≤ Nₖ-1 and a range in the l direction set to 0 ≤ l ≤ Nₗ-1 is used (Nₖ and Nₗ are natural numbers). As the window function Wa (k, 1), a Hamming window, a Hanning window, a Blackman window, or the like can be applied.

When the observation position in the data column x (k, 1) of the magnetic domain image is expressed by an index (n, m), and the shift amounts of the window function Wa (k, l) in the k direction and the l direction are expressed as Sₖ and Sₗ, respectively (n, m, Sₖ, and Sₗ are integers.), a data column xₙₘ (k-nSₖ, l-mSₗ) of a partial region obtained by cutting out a range of nSₖ ≤ k ≤ nSₖ + Nₖ-1 and mSₗ ≤ l ≤ mSₗ + Nₗ-1 from the magnetic domain image is obtained as in Expression (1).
[Mathematical Formula 1] ${x}_{nm} \left(k-{nS}_{k},l-{mS}_{l}\right) = {W}_{a} \left(k-{nS}_{k},l-{mS}_{l}\right) x \left(k, l\right)$

FIG. 8 illustrates an example in which partial regions respectively corresponding to the observation positions (n, m) = (1, 1), (2, 2), (3, 3),..., and (P, Q) (P and Q are natural numbers) are cut out from the magnetic domain image G.

In the present embodiment, Nₖ and Nₗ that define the range of the window function Wa (k, 1) are parameters corresponding to the number of pixels in the k direction and the number of pixels in the l direction in the partial region, respectively.

### (A-2) Treatment of performing ST2DFT

When the data column of the partial region is defined as xₙₘ (n', m') = xₙₘ (k-nSₖ, l-mSₗ), and the two-dimensional Fourier transform is performed on xₙₘ (n', m'), a partial Fourier image X (fₖ, fₗ, n, m) corresponding to the partial region of the observation position (n, m) is obtained as in Expression (2).
[Mathematical Formula 2] $X \left({f}_{k}, {f}_{l}, n, m\right) = {\sum }_{n ′ = 0}^{{N}_{k} - 1} {\sum }_{m ′ = 0}^{{N}_{l} - 1} {x}_{nm} \left(n′,m′\right) exp \left\{-2πj\left(\frac{{f}_{k} n ′}{{N}_{k}}+\frac{{f}_{l} m ′}{{N}_{l}}\right)\right\}$

Here, fₖ and fₗ are space frequencies.

When the resolution of the space frequency fₖ is denoted by Δfₖ and the resolution of the space frequency fₗ is denoted by Δfₗ, Δfₖ and Δfₗ are defined as in Expression (3).
[Mathematical Formula 3] $\left\{\begin{matrix}Δ {f}_{k} = \frac{2}{{N}_{k} Δ k} \\ Δ {f}_{l} = \frac{2}{{N}_{l} Δ l}\end{matrix}\right.$

Δk and Δl are the space resolution in the k direction and the space resolution in the l direction in the magnetic domain image, respectively.

For example, when the two-dimensional Fourier transform is performed on the data column xₙₘ (k-nSₖ, l-mSₗ) of each partial region illustrated in FIG. 8, a partial Fourier image X (fₖ, fₗ, n, m) is obtained for each observation position (n, m) as illustrated in FIG. 9.

### (A-3) Treatment of deriving distribution of spacing of magnetic domain walls

When the partial Fourier image X (fₖ, fₗ, n, m) is obtained, the coordinates (k component fₖ^{max} (n, m) and l component fₗ^{max} (n, m)) of the peak position of the spot of the partial Fourier image X (fₖ, fₗ, n, m) are obtained. Regarding the derivation of the peak position, a region in the vicinity of k = 0 and 1 = 0 is a part that greatly depends on the contrast of the image, and thus is excluded.

Then, the distribution L (n, m) of the spacing of magnetic domain walls is derived as in Expression (4) from the resolution of the space frequency defined by Expression (3) and the peak position of the spot of the partial Fourier image.
[Mathematical Formula 4] $L \left(n, m\right) = \frac{1}{\sqrt{{\left(Δ{f}_{k}{f}_{k}^{max}\left(n, m\right)\right)}^{2} + {\left(Δ{f}_{l}{f}_{l}^{max}\left(n, m\right)\right)}^{2}}}$

As described above, by using ST2DFT, it is possible to quantitatively derive the distribution L (n, m) of the spacing of magnetic domain walls while maintaining the position information of the magnetic domain image.

When the calculation unit 41 derives the distribution of the spacings of magnetic domain walls, the calculation unit 41 determines the region where the spacings of magnetic domain walls are the predetermined value or more as the treatment region (that is, a region to which the magnetic domain control treatment is applied). The control unit 513 of the laser irradiation device 500 controls to turn on the power of the laser beam LB with respect to the treatment region, and preferably to turn off the power of the laser beam LB with respect to the region other than the treatment region. As a result, the magnetic domain control treatment line 11 is introduced into the treatment region of the original sheet. In the other regions, introduction of the magnetic domain control treatment line 11 is suppressed.

The magnetic domain image of the grain-oriented electrical steel sheet 1 after the magnetic domain control treatment can also be obtained by the above-described procedure. In the magnetic domain image of the grain-oriented electrical steel sheet 1, the magnetic domain control treatment line 11 may be unclear. In this case, the observation conditions may be adjusted so that the magnetic domain control treatment line 11 can be clearly confirmed. For example, the magnetic domain control treatment line 11 can be clarified by applying a DC magnetic field along the sheet surface perpendicular direction (thickness direction) of the grain-oriented electrical steel sheet 1.

### (Insulating Coating Forming Step)

In a case where an insulating coating is formed on the surface of the grain-oriented electrical steel sheet, an insulating coating forming step of forming an insulating coating by a known method after final annealing may be included. The insulating coating forming step may be performed before the magnetic domain control treatment line forming step or may be performed after the magnetic domain control treatment line forming step as long as the step is performed after the final annealing. However, when the insulating coating is formed before the magnetic domain control treatment line forming step, the insulating coating may be peeled off in the magnetic domain control treatment line 11. Therefore, the step is preferably performed after the magnetic domain control treatment line forming step. In a case where the insulating coating forming step is performed before the magnetic domain control treatment line forming step, the insulating coating is preferably formed again on the magnetic domain control treatment line 11 after the magnetic domain control treatment line forming step. Examples

The effects of the aspects of the present invention will be described more specifically with reference to Examples. However, the conditions in the examples are merely one condition example adopted to confirm the operability and effects of the present invention. The present invention is not limited to this one condition example. The present invention can adopt various conditions as long as the object of the present invention is achieved without departing from the gist of the present invention. A grain-oriented electrical steel sheet of the same lot having a sheet thickness of 0.20 mm was used as the original sheet. This grain-oriented electrical steel sheet had a base steel sheet containing 3.40% of Si, a forsterite film, and an insulating coating.

The grain-oriented electrical steel sheets No. 1 to 35 were cut out from the grain-oriented electrical steel sheets, and magnetic domain images of the surfaces of the grain-oriented electrical steel sheets (magnetic domain images before magnetic domain control treatment) were acquired. Based on the obtained magnetic domain image, the distribution of the spacing of magnetic domain walls in the grain-oriented electrical steel sheet was acquired, and the region where the spacing of magnetic domain walls was more than 500 µm was specified.

Thereafter, the magnetic domain control treatment was performed on each grain-oriented electrical steel sheet (original sheet) under various conditions. At that time, a procedure of forming the magnetic domain control treatment line is shown in Table 1. The directions, intervals, and types of the formed magnetic domain control treatment lines were as shown in Table 2. In a case where the thermal strains and grooves were formed, the ratio was set to approximately 1 : 1 in terms of the total length.

Thereafter, a magnetic domain image (magnetic domain image after magnetic domain control treatment) of the surface of the grain-oriented electrical steel sheet after formation of the magnetic domain control treatment line was acquired, and distribution of the spacing of magnetic domain walls was acquired from this magnetic domain image.

Using the magnetic domain image before the magnetic domain control treatment and the magnetic domain image after the magnetic domain control treatment, a region larger than a spacing of magnetic domain walls derived from the magnetic domain image after the magnetic domain control treatment by 100 µm or more was defined as a first region, and other regions were defined as a second region, and a linear density of the magnetic domain control treatment line in the second region in mm/mm² was compared with a linear density of the magnetic domain control treatment line in the first region in mm/mm².

As a result of the comparison, the relationship between the linear density of the second region and the linear density of the first region is shown in Table 1. In the table, OK indicates that the linear density of the second region is smaller than the linear density of the first region, and NG indicates that the linear density of the second region is larger than the linear density of the first region, or the linear density of the second region is the same as the linear density of the first region.

Subsequently, magnetic domain control treatment lines were further formed (additional magnetic domain control treatment lines were formed) for some examples. At that time, a magnetic domain control treatment line was formed in the first region.

For the example in which the additional magnetic domain control treatment line was formed, the linear density of the first region and the linear density of the second region were compared. As a result of the comparison, the relationship between the linear density of the second region and the linear density of the first region is shown in Table 1. In the table, OK indicates that the linear density of the second region is smaller than the linear density of the first region, and NG indicates that the linear density of the second region is larger than the linear density of the first region, or the linear density of the second region is the same as the linear density of the first region.

Thus, a grain-oriented electrical steel sheet was produced.

For the obtained grain-oriented electrical steel sheet, in a case where the magnetic domain control treatment line was the thermal strain, the absolute maximum value of the tensile stress in an arbitrary direction in the magnetic domain control treatment line was measured. The results are illustrated in Table 2.

In addition, a sample having a size of 100 mm × 100 mm was collected from the obtained grain-oriented electrical steel sheet, a first magnetic domain image of the surface of the sample was obtained using an image acquisition device including a light source unit, a magneto-optical sensor (MO sensor), an image sensor, and a signal processing unit, and the spacing of magnetic domain walls and the linear density of the magnetic domain control treatment line were measured.

In addition, this sample was annealed by retaining at 800°C for 240 minutes, cooling to 200°C at an average cooling rate of 25°C/h up to 50°C and then 100°C/h, magnetized to a magnetic flux density of 1.9 T (so that the magnetic flux density was 1.9 T) by applying an AC magnetic field, and demagnetized by attenuating the AC magnetic field.

Thereafter, a second magnetic domain image was obtained on this sample in the same manner as the position where the first magnetic domain image was obtained, and the spacing of magnetic domain walls and the linear density of the magnetic domain control treatment line were measured.

The results are shown in Table 3.

The noise characteristics and iron loss of the obtained grain-oriented electrical steel sheet were evaluated as follows. The results are shown in Table 3.

### [Noise Characteristics]

The methods for evaluating noise characteristics and iron loss were as follows.

A three-phase transformer core is prepared by laminating 205 sheets of the obtained grain-oriented electrical steel sheets having a sheet thickness of 0.20 mm. In the production, the widths of the leg and the yoke of the three-phase transformer core were both 150 mm. The height and width of the outer shape of the three-phase transformer core were both 750 mm. Noise and iron loss of these three-phase transformer cores were measured. The measurement conditions were a frequency of 60 Hz and an excitation magnetic flux density of 1.7 T.

In measuring the noise, microphones were arranged at equal intervals at eight points around the transformer in which the three-phase transformer core was incorporated. The distance between the transformer and the microphone was 30 cm. A noise evaluation result (unit: dBA) of the grain-oriented electrical steel sheet was a value obtained by correcting A characteristics to the noise measurement result by the microphone and averaging the results. An example in which the evaluation result of noise was 37.00 dBA or less was determined to be an example in which noise reduction was achieved.

### [Iron loss]

The iron loss was obtained by measuring voltages and currents on the primary side and the secondary side with a power analyzer when excitation was performed at a frequency of 60 Hz and an excitation magnetic flux density of 1.7 T as described above. The obtained iron loss is described in Table 3 as an iron loss evaluation result (unit: W/kg) of the grain-oriented electrical steel sheet. An example in which the evaluation result of the iron loss was 1.03 W/kg or less was determined to be an example in which iron loss reduction was achieved.

As shown in Tables 1 to 3, in the invention examples, the linear density of the second region was smaller than the linear density of the first region, and both the iron loss and the noise were suppressed to be low. In particular, in a case where the difference between the linear density of the second region and the linear density of the first region was large, the iron loss was lower. In a case where the magnetic domain control treatment lines were grooves and thermal strains, noise was lower.

On the other hand, in the comparative example, the linear density of the second region was not smaller than the linear density of the first region, and one or both of the iron loss and the noise were high.

**[Table 1]**

| No. | Magnetic domain control treatment line forming step | Magnetic domain image comparison step | Additional magnetic domain control treatment line forming step | Magnetic domain image comparison step (After additional magnetic domain control treatment line forming step) |
|---|---|---|---|---|
| 1 | Form straight linear magnetic domain control treatment line mainly in region in which spacing of magnetic domain walls is more than 500 µm | OK | - | - |
| 2 | Form straight linear magnetic domain control treatment line mainly in region in which spacing of magnetic domain walls is more than 500 µm | OK | - | - |
| 3 | Form straight linear magnetic domain control treatment line mainly in region in which spacing of magnetic domain walls is more than 500 µm | OK | - | - |
| 4 | Form straight linear magnetic domain control treatment line mainly in region in which spacing of magnetic domain walls is more than 500 µm | NG | Implementation | OK |
| 5 | Form straight linear magnetic domain control treatment line mainly in region in which spacing of magnetic domain walls is more than 500 µm | NG | Implementation | OK |
| 6 | Form straight linear magnetic domain control treatment line mainly in region in which spacing of magnetic domain walls is more than 500 µm | OK | - | - |
| 7 | Form straight linear magnetic domain control treatment line mainly in region in which spacing of magnetic domain walls is more than 500 µm | NG | Implementation | OK |
| 8 | Form straight linear magnetic domain control treatment line mainly in region in which spacing of magnetic domain walls is more than 500 µm | OK | - | - |
| 9 | Form straight linear magnetic domain control treatment line mainly in region in which spacing of magnetic domain walls is more than 500 µm | OK | - | - |
| 10 | Form straight linear magnetic domain control treatment line mainly in region in which spacing of magnetic domain walls is more than 500 µm | OK | - | - |
| 11 | Form straight linear magnetic domain control treatment line mainly in region in which spacing of magnetic domain walls is more than 500 µm | OK | - | - |
| 12 | Form straight linear magnetic domain control treatment line mainly in region in which spacing of magnetic domain walls is more than 500 µm | NG | Implementation | OK |
| 13 | Form straight linear magnetic domain control treatment line mainly in region in which spacing of magnetic domain walls is more than 500 µm | NG | Implementation | OK |
| 14 | Form straight linear magnetic domain control treatment line mainly in region in which spacing of magnetic domain walls is more than 500 µm | NG | Implementation | OK |
| 15 | Form straight linear magnetic domain control treatment line mainly in region in which spacing of magnetic domain walls is more than 500 µm | OK | - | - |
| 16 | Form straight linear magnetic domain control treatment line mainly in region in which spacing of magnetic domain walls is more than 500 µm | OK | - | - |
| 17 | Form straight linear magnetic domain control treatment line mainly in region in which spacing of magnetic domain walls is more than 500 µm | OK | - | - |
| 18 | Form straight linear magnetic domain control treatment line mainly in region in which spacing of magnetic domain walls is more than 500 µm | OK | - | - |
| 19 | Form straight linear magnetic domain control treatment line mainly in region in which spacing of magnetic domain walls is more than 500 µm | OK | - | - |
| 20 | Form straight linear magnetic domain control treatment line mainly in region in which spacing of magnetic domain walls is more than 500 µm | NG | Implementation | OK |
| 21 | Form straight linear magnetic domain control treatment line mainly in region in which spacing of magnetic domain walls is more than 500 µm | OK | - | - |
| 22 | Form straight linear magnetic domain control treatment line mainly in region in which spacing of magnetic domain walls is more than 500 µm | OK | - | - |
| 23 | Form straight linear magnetic domain control treatment line mainly in region in which spacing of magnetic domain walls is more than 500 µm | OK | - | - |
| 24 | Form straight linear magnetic domain control treatment line mainly in region in which spacing of magnetic domain walls is more than 500 µm | OK | - | - |
| 25 | Form straight linear magnetic domain control treatment line mainly in region in which spacing of magnetic domain walls is more than 500 µm | OK | - | - |
| 26 | Form straight linear treatment line over entire width of sample | NG | - | - |
| 27 | Form random broken linear treatment line | NG | - | - |
| 28 | Form regular broken linear treatment line | NG | - | - |
| 29 | Form regular broken linear treatment line | NG | - | - |
| 30 | Form magnetic domain cont^{r}ol treatment line mainly in region in which spacing of magnetic domain walls is more than 500 µm | NG | - | - |
| 31 | Form magnetic domain control treatment line mainly in region in which spacing of magnetic domain walls is more than 500 µm | NG | Implementation | NG |
| 32 | Six magnetic domain control treatment lines with an interval of 4 mm in the rolling direction were formed in the central region in the rolling direction of the grains with the radius of curvature R = 300 mm at the time of finish annealing. | NG | - | - |
| 33 | Six magnetic domain control treatment lines with an interval of 4 mm in the rolling direction were formed in the central region in the rolling direction of the grains with the radius of curvature R = 300 mm at the time of finish annealing. | OK | - | - |
| 34 | Form linear magnetic domain control treatment line including mainly curve in region in which spacing of magnetic domain walls is more than 500 µm | OK | - | - |
| 35 | Form linear magnetic domain control treatment line including mainly curve in region in which spacing of magnetic domain walls is more than 500 µm | OK | - | - |

**[Table 2]**

| No. | Magnetic domain control treatment line | | | | | |
|---|---|---|---|---|---|---|
| | Angle formed with transverse direction (°) | Interval in rolling direction (mm) | Type (Groove of thermal strain) | Average width of groove (µm) | Average depth of groove (µm) | Absolute maximum value of tensile stress of cross section passing through magnetic domain control treatment line (MPa) |
| 1 | 0 | 5 | Thermal strain | - | - | 38 |
| 2 | 0 | 5 | Thermal strain | - | - | 42 |
| 3 | 0 | 5 | Thermal strain | - | - | 187 |
| 4 | 5 | 5 | Thermal strain | - | - | 152 |
| 5 | 5 | 2 | Thermal strain | - | - | 145 |
| 6 | 5 | 2 | Thermal strain | - | - | 145 |
| 7 | 5 | 4 | Thermal strain | - | - | 198 |
| 8 | 5 | 8 | Thermal strain | - | - | 211 |
| 9 | 5 | 10 | Thermal strain | - | - | 167 |
| 10 | 5 | 15 | Thermal strain | - | - | 143 |
| 11 | 10 | 5 | Thermal strain | - | - | 164 |
| 12 | 30 | 5 | Thermal strain | - | - | 187 |
| 13 | 45 | 5 | Thermal strain | - | - | 105 |
| 14 | 5 | 5 | Thermal strain | - | - | 154 |
| 15 | 5 | 5 | Thermal strain | - | - | 123 |
| 16 | 5 | 5 | Groove + thermal strain | 20 | 5 | 167 |
| 17 | 5 | 6 | Groove + thermal strain | 20 | 10 | 182 |
| 18 | 5 | 5 | Groove + thermal strain | 20 | 35 | 204 |
| 19 | 5 | 5 | Groove + thermal strain | 20 | 45 | 245 |
| 20 | 5 | 4 | Groove + thermal strain | 20 | 10 | 235 |
| 21 | 5 | 5 | Groove + thermal strain | 10 | 10 | 183 |
| 22 | 5 | 5 | Groove + thermal strain | 50 | 10 | 196 |
| 23 | 5 | 5 | Groove + thermal strain | 150 | 10 | 165 |
| 24 | 5 | 5 | Groove + thermal strain | 300 | 10 | 174 |
| 25 | 5 | 5 | Groove + thermal strain | 20 | 35 | 177 |
| 26 | 5 | 5 | Thermal strain | - | - | 192 |
| 27 | 5 | 5 | Thermal strain | - | - | 192 |
| 28 | 5 | 5 | Thermal strain | - | - | 38 |
| 29 | 5 | 5 | Groove + thermal strain | 20 | 5 | 164 |
| 30 | 0 | 5 | Thermal strain | - | - | 180 |
| 31 | 0 | 5 | Thermal strain | - | - | 220 |
| 32 | 5 | 5 | Thermal strain | - | - | 123 |
| 33 | 5 | 5 | Groove + thermal strain | 20 | 35 | 144 |
| 34 | 5 | 5 | Thermal strain | - | - | 181 |
| 35 | 5 | 5 | Groove + thermal strain | 20 | 35 | 177 |

**[Table 3]**

| No. | Linear density of magnetic domain control treatment line in first region (mm/mm²) | Linear density of magnetic domain control treatment line in second region (mm/mm²) | Difference in linear density (Linear density of second region - linear density of first region) (mm/mm²) | Characteristics | | Remarks |
|---|---|---|---|---|---|---|
| | | | | Iron loss (W/Kg) | Noise characteristics (dBA) | |
| 1 | 0.21 | 0.11 | -0.10 | 1.03 | 35.16 | Invention Example |
| 2 | 0.21 | 0.03 | -0.18 | 1.01 | 35.03 | Invention Example |
| 3 | 0.25 | 0.04 | -0.21 | 0.98 | 34.20 | Invention Example |
| 4 | 0.28 | 0.12 | -0.16 | 0.97 | 35.70 | Invention Example |
| 5 | 0.62 | 0.38 | -0.24 | 0.93 | 36.57 | Invention Example |
| 6 | 0.62 | 0.42 | -0.20 | 0.93 | 36.95 | Invention Example |
| 7 | 0.42 | 0.22 | -0.20 | 0.95 | 36.51 | Invention Example |
| 8 | 0.16 | 0.01 | -0.15 | 1.00 | 33.42 | Invention Example |
| 9 | 0.13 | 0.02 | -0.11 | 1.02 | 33.31 | Invention Example |
| 10 | 0.08 | 0.06 | -0.02 | 1.03 | 32.87 | Invention Example |
| 11 | 0.15 | 0.13 | -0.02 | 0.95 | 34.26 | Invention Example |
| 12 | 0.22 | 0.10 | -0.12 | 0.95 | 34.20 | Invention Example |
| 13 | 0.27 | 0.12 | -0.15 | 0.94 | 34.69 | Invention Example |
| 14 | 0.31 | 0.04 | -0.27 | 0.94 | 33.39 | Invention Example |
| 15 | 0.34 | 0.01 | -0.33 | 0.94 | 32.98 | Invention Example |
| 16 | 0.15 | 0.05 | -0.10 | 0.98 | 34.25 | Invention Example |
| 17 | 0.32 | 0.16 | -0.16 | 0.97 | 33.87 | Invention Example |
| 18 | 0.22 | 0.15 | -0.07 | 1.01 | 32.88 | Invention Example |
| 19 | 0.21 | 0.16 | -0.05 | 1.01 | 32.48 | Invention Example |
| 20 | 0.27 | 0.18 | -0.09 | 0.98 | 33.87 | Invention Example |
| 21 | 0.12 | 0.10 | -0.02 | 1.02 | 32.02 | Invention Example |
| 22 | 0.24 | 0.11 | -0.13 | 0.99 | 33.41 | Invention Example |
| 23 | 0.21 | 0.05 | -0.16 | 1.00 | 33.02 | Invention Example |
| 24 | 0.26 | 0.07 | -0.19 | 0.98 | 32.97 | Invention Example |
| 25 | 0.37 | 0.00 | -0.37 | 0.96 | 32.15 | Invention Example |
| 26 | 0.25 | 0.25 | 0.00 | 0.98 | 38.20 | Comparative Example |
| 27 | 0.12 | 0.30 | 0.18 | 1.06 | 36.02 | Comparative Example |
| 28 | 0.21 | 0.28 | 0.07 | 1.05 | 37.94 | Comparative Example |
| 29 | 0.18 | 0.22 | 0.04 | 0.99 | 38.10 | Comparative Example |
| 30 | 0.11 | 0.12 | 0.01 | 1.09 | 34.50 | Comparative Example |
| 31 | 0.22 | 0.23 | 0.01 | 0.97 | 38.80 | Comparative Example |
| 32 | 0.17 | 0.17 | 0.00 | 1.08 | 33.00 | Comparative Example |
| 33 | 0.17 | 0.17 | 0.00 | 1.09 | 32.80 | Comparative Example |
| 34 | 0.37 | 0.01 | -0.36 | 0.91 | 31.88 | Invention Example |
| 35 | 0.39 | 0.00 | -0.39 | 0.92 | 31.52 | Invention Example |

### INDUSTRIAL APPLICABILITY

According to the present disclosure, it is possible to provide a grain-oriented electrical steel sheet having a low iron loss (low iron loss) and having a low noise (excellent noise characteristics) when the grain-oriented electrical steel sheet is made into an electrical product, and a method for manufacturing the grain-oriented electrical steel sheet. Therefore, industrial applicability is high.

### REFERENCE SIGNS LIST

1 Grain-oriented electrical steel sheet
11 Magnetic domain control treatment line
21 First region
22 Second region
RD Rolling direction
TD Transverse direction (sheet width direction)
ND Rolling surface normal direction
30 Image acquisition device
31 Light source unit
33 MO sensor
35 Image sensor
37 Signal processing unit
40 Analysis device
41 Calculation unit
43 Memory
45 Display unit
47 Input unit
49 Communication I/F
301 Flux closure domain
302 Noise
Ls Line segment
Ip Intersection point
500 Laser irradiation device
501 Polygon mirror
503 light source device
505 Collimator
507 Condenser lens
509 Motor
511 Sensor
513 Control unit
515 Sheet passing device

## Claims

1. A grain-oriented electrical steel sheet having a surface on which a plurality of magnetic domain control treatment lines extending in a direction intersecting a rolling direction are formed, wherein
a magnetic domain image of the surface is defined as a first magnetic domain image,
a magnetic domain image at the same position as that of the first magnetic domain image after the grain-oriented electrical steel sheet is annealed so as to be retained at 800°C for 240 minutes or more, cooled to 200°C at an average cooling rate of 25°C/h or less, and then cooled to 50°C or less at an average cooling rate of 100°C/h or less, is magnetized to a magnetic flux density of 1.9 T or more by applying an AC magnetic field, and is demagnetized by attenuating the AC magnetic field is defined as a second magnetic domain image, and
when a region in which a spacing of magnetic domain walls derived from the second magnetic domain image is larger than a spacing of magnetic domain walls derived from the first magnetic domain image by 100 µm or more is defined as a first region, and other regions are defined as a second region,
a linear density of the magnetic domain control treatment line in the second region in mm/mm² is smaller than a linear density of the magnetic domain control treatment line in the first region in mm/mm².

2. The grain-oriented electrical steel sheet according to claim 1, wherein
a difference between the linear density of the magnetic domain control treatment line in the second region and the linear density of the magnetic domain control treatment line in the first region is 0.20 mm/mm² or more.

3. The grain-oriented electrical steel sheet according to claim 1 or 2, wherein
the plurality of magnetic domain control treatment lines are thermal strains, or grooves and the thermal strains.

4. The grain-oriented electrical steel sheet according to claim 1 or 2, wherein
the plurality of magnetic domain control treatment lines are thermal strains into which a tensile stress of 40 MPa or more is introduced.

5. A method for manufacturing a grain-oriented electrical steel sheet, the method comprising:
a first magnetic domain image acquisition step of acquiring a magnetic domain image before magnetic domain control treatment on a surface of a grain-oriented electrical steel sheet;
a spacing of magnetic domain walls distribution acquisition step of acquiring a distribution of a spacing of magnetic domain walls in the grain-oriented electrical steel sheet based on the magnetic domain image before magnetic domain control treatment obtained in the first magnetic domain image acquisition step;
a magnetic domain control treatment line forming step of forming a magnetic domain control treatment line on the surface of the grain-oriented electrical steel sheet;
a second magnetic domain image acquisition step of acquiring a magnetic domain image after magnetic domain control treatment on the surface of the grain-oriented electrical steel sheet on which the magnetic domain control treatment line is formed;
a magnetic domain image comparison step of comparing the magnetic domain image before the magnetic domain control treatment with the magnetic domain image after the magnetic domain control treatment; and
an additional magnetic domain control treatment line forming step of further forming a magnetic domain control treatment line on the surface of the grain-oriented electrical steel sheet after the magnetic domain image comparison step as necessary,
wherein
in the magnetic domain control treatment line forming step,
the magnetic domain control treatment line is formed in a region where the spacing of magnetic domain walls is more than 500 µm based on the distribution of the spacing of magnetic domain walls obtained in the spacing of magnetic domain walls distribution acquisition step,
in the magnetic domain image comparison step,
when a region in which a spacing of magnetic domain walls derived from the magnetic domain image before the magnetic domain control treatment is larger than a spacing of magnetic domain walls derived from the magnetic domain image after the magnetic domain control treatment by 100 µm or more is defined as a first region, and other regions are defined as a second region, a linear density of the magnetic domain control treatment line in the second region in a unit of mm/mm² is compared with a linear density of the magnetic domain control treatment line in the first region in a unit of mm/mm², and
in the additional magnetic domain control treatment line forming step,
the magnetic domain control treatment line is formed in the first region in a case where the linear density of the second region is equal to or larger than the linear density of the first region, and
the second magnetic domain image acquisition step, the magnetic domain image comparing step, and the additional magnetic domain control treatment line forming step are repeated until the linear density of the magnetic domain control treatment line in the second region becomes smaller than the linear density of the magnetic domain control treatment line in the first region.

6. The method for manufacturing a grain-oriented electrical steel sheet according to claim 5, wherein
in the magnetic domain control treatment line forming step, the magnetic domain control treatment line is formed by irradiation with a laser or an electron beam.
